

# UNITED STATES PATENT OFFICE.

FRANZ STEIMMIG, OF HANOVER, GERMANY.

## PROCESS OF PRECIPITATING VISCOSE.

1,399,587.

Specification of Letters Patent.

Patented Dec. 6, 1921.

No Drawing. Original application filed June 12, 1913, Serial No. 773,324. Divided and this application filed August 12, 1916. Serial No. 114,661.

(GRANTED UNDER THE PROVISIONS OF THE ACT OF MARCH 3, 1921, 41 STAT. L., 1313.)

*To all whom it may concern:*

Be it known that I, FRANZ STEIMMIG, a subject of the German Empire, residing at Hanover, Germany, have invented certain new and useful Improvements in Processes of Precipitating Viscose, (for which I have filed applications in Germany, Feb. 15, 1913, and Great Britain May 10, 1913,) of which the following is a specification.

10 This invention relates to the production of cellulose compounds suitable for use as films or filaments for fabrics from the material known commercially as "viscose" which is produced from a solution of cellulose as described in U. S. Patent No. 520770 dated June 5th, 1894.

In the manufacture of threads suitable for the manufacture of yarns and fabrics from viscose, preference has been given to 20 setting baths consisting of acidulated solutions. This is readily understood in view of the fact that viscose contains a cellulose derivative which is soluble in an alkaline solution, that is to say, it cannot be precipitated by being acted upon by an alkali.

Nevertheless it would be advantageous to employ a setting bath with an alkaline action for cellulose derivatives produced from viscose. It is known that viscose may be 30 coagulated by the aid of a concentrated solution of a neutral salt, (Patent No. 520770 of 1894.) This coagulating action cannot, however, be employed commercially in a satisfactory manner to produce derivatives 35 of cellulose with continuous operation of the process owing to the fact that the increasing quantity of alkali in the bath soon renders its presence felt by preventing the coagulation.

40 I have discovered that an excellent setting bath may be made with a solution of such neutral salts by adding a certain quantity of an ammonium salt to the same, for instance ammonium sulfate. Excellent results have been obtained with a precipitating bath made with a concentrated solution of sodium sulfate to which about 10% of ammonium sulfate is added. This result is somewhat unexpected as in view of the experience gained with the process described 45 in U. S. Patent No. 622087 dated 28th March, 1899, it would appear that only a

concentrated solution (say 30% to 40%) of ammonium sulfate would provide an effective setting bath, that is to say a solution 55 containing about three to four times as much ammonium sulfate as the solution mentioned above. It should also be remembered that it is impossible with ordinary commercial viscose to precipitate a single 60 filament with a ten per cent. ordinary solution of ammonium sulfate.

In making the setting bath, I preferably prepare a solution containing ammonium sulfate, and a neutral salt such as sodium 65 sulfate (Glauber's salt), magnesium chlorid, calcium chlorid, or sodium chlorid. In place of such neutral salts, I can also employ such a material as a tertiary alcohol, *e. g.* glycerin. 70

The quantity of ammonium salt to be added to the neutral salt solution such as brine may be varied within narrow limits only. The amount depends to a great extent upon the kind of product which it is desired to 75 produce and would require to be different in the case of coarse fibers, say imitation horse hair and in the case of fine fibers such as are necessary for artificial silk. The best amount to add should be found by trial in 80 every case, but it should be retained as low as possible in the interests of cheapness.

It is preferable to use in conjunction with my improved precipitating bath some third substance, (such as an oxidizing agent or a 85 reducing salt) just as in the case of acid baths. These agents, which may be sugar, arsenous compounds or the like, (which act as reducing agents) or sodium hypochlorite (which acts as an oxidizing agent) have the 90 effect of adding brilliancy to the fibers. It is also quite practical to add metal salts to the precipitating bath as is known in another process, which salts form insoluble sulfids with the alkaline sulfid. This latter 95 method is not however necessary as experience shows that with the herein described new bath there is no tendency of the fibers to become sticky.

The filaments or films may be squirted in 100 any suitable way into the precipitating bath and on leaving this they are wound preferably on a drum which rotates in brine. In this way the cellulose derivatives are washed,

whereupon they are preferably suitably fixed in acid and washed in water and finally dried.

The further treatment of the filaments or 5 films proceeds in the usual manner. The process not only results in greater cheapness, but a further characteristic resides in the strength and toughness of the product.

The additional substance herein mentioned, such as the oxidizing, or reducing 10 organic substances are added for known purposes to affect the product and it has been found that with the invention such substances may be used with similar results as 15 obtained in the known coagulating solutions.

In all cases I prefer to employ a setting 20 bath containing one or more of the neutral salts above referred to (NaCl, Na<sub>2</sub>SO<sub>4</sub>, MgCl<sub>2</sub>, CaCl<sub>2</sub>, etc.), which compounds are generically referred to as "a neutral salt" of 25 an alkali-forming metal and also containing a relatively small amount of an ammonium salt, capable of existing in solution with the "neutral salt" (one or more of such) employed. Other agents for the production of special effects may be added if desired. The bath will preferably be substantially saturated with the "neutral salt" 30 employed.

30 I call particular attention to the use of a solution made up by dissolving in thirty parts of water, sixty parts of Glauber's salt (Na<sub>2</sub>SO<sub>4</sub>·10H<sub>2</sub>O) and ten parts of ammonium sulfate. Such a bath has given excellent 35 results, and is preferably maintained at a temperature of 35° to 40° C.

Another bath which I find gives excellent 40 results is a solution containing 19 parts NaCl<sub>1</sub>; 12.5 parts CaCl<sub>2</sub>; 10 parts NH<sub>4</sub>Cl, and 48.5 parts water. Another bath giving 45 excellent results is a solution of 45 parts CaCl<sub>2</sub>; 10 parts NH<sub>4</sub>Cl; and 45 parts of water. Magnesium chlorid in various mixtures gives good results.

45 Regarding the ammonium salt, this may be ammonium sulfate or ammonium chlorid, and I find that a mixture of these two, also gives good results.

I do not claim the setting baths, *per se*, 50 in the present case, since said baths form the subject matter of my copending application 773,324 of which the present case is a division.

What I claim is:—

55 1. Process for treating cellulose products for the manufacture of films and filaments, which consists in squirting the viscose into an acid-free concentrated solution of a neutral salt also containing only a small percentage of an ammonium salt.

60 2. A process of treating viscose which comprises subjecting the same to the action of an acid-free bath containing a neutral salt and about ten per cent. of ammonium sulfate.

3. A process of treating viscose which 70 consists in squirting the same into an acid-free solution containing ammonium sulfate and sodium sulfate.

4. A process for treating viscose which 75 comprises subjecting the same to the action of an acid-free setting bath comprising a solution substantially saturated with a neutral salt, and containing a small percentage only of an ammonium salt.

5. A process of treating viscose which 80 comprises subjecting the same to the action of an acid-free setting bath comprising a solution substantially saturated with a neutral salt, and containing not over 10% of an ammonium salt.

6. A process of treating viscose which 85 comprises subjecting the same to the action of an acid-free setting bath comprising a solution substantially saturated with a neutral salt, and containing not over 10% of an ammonium sulfate.

7. A process of treating viscose which 90 comprises subjecting the same to the action of an acid-free setting bath comprising a solution substantially saturated with sodium sulfate and containing a small percentage only of an ammonium salt.

8. A process of treating viscose which 95 comprises subjecting the same to the action of an acid-free setting bath comprising a solution substantially saturated with sodium sulfate and containing not over 10% of an ammonium salt.

9. A process of treating viscose which 100 comprises subjecting the same to the action of an acid-free setting bath comprising a solution substantially saturated with sodium sulfate and containing not over 10% of an ammonium sulfate.

10. A process of treating viscose which 105 comprises subjecting the same to the action of an acid-free setting bath comprising a solution substantially saturated with sodium sulfate and containing an ammonium salt.

11. A process of treating viscose which 110 comprises subjecting the same to the action of an acid-free setting bath comprising a solution substantially saturated with a neutral salt of an alkali forming metal and containing not over 10% of an ammonium salt.

12. A process of treating viscose which 115 comprises subjecting the same to the action of an acid-free setting bath comprising a solution substantially saturated with a neutral salt of an alkali forming metal and containing a small percentage of an ammonium salt.

13. A process of treating viscose which 120 comprises subjecting the same to the action of an acid-free setting bath comprising a solution substantially saturated with a neutral salt of an alkali forming metal and containing ammonium sulfate.

14. A process of treating viscose which comprises subjecting the same to the action of an acid-free setting bath comprising a solution substantially saturated with sodium sulfate and containing a small percentage of ammonium sulfate.

5 15. A process of treating viscose which comprises subjecting the same to the action of an acid-free setting bath comprising a

solution substantially saturated with sodium sulfate and containing not over 10% of an ammonium sulfate.

In testimony whereof I affix my signature in the presence of two witnesses.

FRANZ STEIMMIG.

Witnesses:

N. N. BEHNE,  
R. MICHAELS.